

## UNITED STATES PATENT OFFICE

HARRY L. HORN, OF NEW YORK, N. Y., ASSIGNOR TO BAGASSE DEVELOPMENT INC., A CORPORATION OF NEW YORK

## METHOD OF PREPARING CELLULOSE PULP

No Drawing.

Application filed December 2, 1929. Serial No. 411,219.

This invention relates to new and useful improvements in a method of preparing cellulose pulp from cellulose bearing material such as bagasse, straws, grasses, wood, corn-stalk and the like.

The invention relates to similar subject matter as disclosed in my copending application, Serial Number 410,702, filed simultaneously with this application.

The invention proposes simultaneous cooking, beating and electrically and chemically treating bagasse, straws, grasses, wood, corn-stalk and the like for forming a pulp capable of being used in well known manner for manufacturing paper, rayon, etc., and which besides distinguishing in the reduction of the cost of the pulp, differs in the production of a higher grade of pulp. It may be obvious that if various steps of a method could be performed simultaneous, that time will be saved, but the producing of a superior product or the possibility of simultaneously performing all of the steps without interference of the steps with each other could not previously be recognized, except by actual trying.

Specific application of the instant invention will be given as it relates to bagasse which is typical of the various cellulose materials previously mentioned. It may be well to call attention that sugar cane is usually cut by a hand cutter a few inches above the ground, because the vegetation of the cane occurs in a junglelike field. After the sugar cane is cut, it is heaped and loaded in a cart and delivered to a factory. The upper part of the cane which forms the leaves and branches is removed and the cane proper is dumped into a crushing machine. The crushing machine has crushing rollers which squeeze out the juice which is used for preparing sugar. The remainder is the bagasse. Millions of tons of this bagasse must be carried away from the sugar mills and destroyed by burning or otherwise.

Numerous attempts have been made to commercially use the bagasse in the production of pulp for the manufacture of paper, rayon and the like, but have failed in that the cost was prohibitive or the product unsatisfactory.

The present invention utilizes this bagasse so that it is possible to refine it and make pulp of good quality cheaply and on a commercial basis.

The pulp produced may be used for making paper, rayon or the like, by methods which are well known. For example, one method is cited which consists in feeding the pulp as obtained from the crusher to a conveyor, drying out the moisture from the pulp by a suitable suction device beneath the conveyor and spreading the pulp into paper sheets after the removal of the moisture. It is necessary to refine the pulp before feeding it to the conveyor by various treatments and coloring to conform with particular requirements. The paper may be manufactured to be of different grades depending upon the quality or thickness of the fibres in the pulp which is of cottonlike texture.

The above method of making paper is conventional, but the particular transforming of the bagasse into pulp as follows, is new. The shredded bagasse as obtained from the crusher must first be washed for removing various impurities such as the remains of the juice dirt, sand and other foreign matter, and then must be fed into a container which is generally known as a digest or by means of a conveyor or thru a manhole. Water is supplied into the conveyor with the shredded bagasse preferably a sufficient amount to cover all of the latter element. A plurality of rods are loosely located in the bottom part of the digestor so that upon rotation these rods may move around and accomplish proper beating of the shredded bagasse.

These rods may be round or of any other suitable shape and may be formed with depressions, slots, grooves or the like.

Sodium chloride is added to the water in the digestor and one terminal of an electric source is connected at one end of the digestor and the other terminal to the other end. The current is then passed thru the liquid in the digestor and electrolytical and chemical action takes place forming sodium hydroxide and chlorine, and simultaneously the digestor is rotated by mechanical means for about two hours. This treatment constitutes a power-

ful softening agent for the shredded bagasse. It is advisable that 10 pounds of sodium chloride be added to 100 pounds of shredded bagasse in 100 gallons of water.

- 5 After two hours of rotation, the digestor is stopped and lime and soda ash is added. Then the digestor is again rotated and simultaneously steam is supplied within it at a pressure of from thirty to fifty pounds. The 10 digestor is now allowed to rotate for a period of from one to two hours. During this period, the steam cooks the contents of the digestor and adds to the softening of the bagasse. Preferably the digestor should rotate at eighteen 15 revolutions per minute. When the machine is stopped, the material is dumped into a container and the juice or water drains off. The resultant matter is the pulp which is to be used in the preparation of paper, rayon and 20 the like by any conventional method. The juice or water may be used for the recovery of by-products such as fertilizers, etc.

The invention method eliminates the necessity of many operations. It eliminates the 25 beating of the pulp either partially or completely and the result is far more efficient than if pulp would be produced by separate steps since cooking, beating, electrical and chemical processes all take place simultaneously 30 and in united action more efficiently and thoroughly accomplish their results than if they were acting singularly.

While I have described my invention with some degree of particularity, I realize that 35 in practice various alterations therein may be made. I therefore reserve the right and privilege of changing the form of the details or otherwise altering the arrangement of the correlated parts without departing from the 40 spirit or the scope of the appended claims.

Having thus described my invention, what I claim as new, and desire to secure by 45 United States Letters Patent is:—

1. A method for preparing cellulose pulp 50 from cellulose bearing material such as bagasse, straws, grasses, wood, cornstalk and the like, consisting in simultaneously cooking, beating and electrically and chemically treating the cellulose bearing material.

55 2. A method for preparing cellulose pulp from cellulose bearing material such as bagasse, straws, grasses, wood, cornstalk, and the like, consisting in simultaneously cooking, beating and electrically and chemically treating the cellulose bearing material, said cooking being accomplished by the introduction of steam into a digestor rotating and carrying the cellulose bearing material in water.

60 3. A method for preparing cellulose pulp from cellulose bearing material such as bagasse, straws, grasses, wood, cornstalk, and the like, consisting in simultaneously cooking, beating and electrically and chemically treating the cellulose bearing material, said cooking 65 being accomplished by the introduction

of steam into a digestor rotating and carrying the cellulose bearing material in water, said beating being accomplished by loose rods within the digestor.

4. A method for preparing cellulose pulp 70 from cellulose bearing material such as bagasse, straws, grasses, wood, cornstalk and the like, consisting in simultaneously cooking, beating and electrically and chemically treating the cellulose bearing material, said cooking being accomplished by the introduction of steam into a digestor rotating and carrying the cellulose bearing material in water, 75 said electrical and chemical treatment consists in passing a current thru said water to which sodium chloride has been previously added.

5. A method for preparing cellulose pulp 80 from cellulose bearing material such as bagasse, straws, grasses, wood, cornstalk and the like, consisting in simultaneously cooking, beating and electrically and chemically treating the cellulose bearing material, said cooking being accomplished by the introduction 85 of steam into a digestor rotating and carrying the cellulose bearing material in water, said electrical and chemical treatment consists in passing a current thru said water to which sodium chloride has been previously 90 added, and at a later period adding lime and soda ash.

6. A method of preparing cellulose pulp 95 from cellulose bearing material, comprising simultaneously cooking, beating and electrically and chemically treating the material, said chemical treatment including the use of a softening agent.

In testimony whereof I have affixed my signature.

HARRY L. HORN.

105

110

115

120

125

130